

[54] FROTH FLOTATION METHOD FOR THE RECOVERY OF MINERALS BY MEANS OF QUATERNARY PHOSPHONIUM NITRITES AND TERNARY PHOSPHINE DINITRITES

[76] Inventor: Vojislav Petrovich, 1925 W. Schiller St., Chicago, Ill. 60622  
[22] Filed: Apr. 23, 1975  
[21] Appl. No.: 570,568

[52] U.S. Cl. .... 209/166  
[51] Int. Cl.<sup>2</sup> .... B03D 1/02  
[58] Field of Search. .... 209/166, 167, 1

[56] References Cited

UNITED STATES PATENTS

|           |         |            |           |
|-----------|---------|------------|-----------|
| 1,552,936 | 9/1925  | McArthur   | 209/167   |
| 2,084,413 | 6/1937  | Siems      | 209/166   |
| 2,132,902 | 10/1938 | Lenher     | 209/166   |
| 2,242,224 | 5/1941  | Bley       | 209/166 X |
| 2,403,640 | 7/1946  | Cunningham | 209/167   |
| 2,861,687 | 11/1958 | Lord       | 209/167   |
| 2,904,177 | 9/1959  | Michal     | 209/167   |
| 2,970,688 | 2/1961  | Uhland     | 209/166   |

3,238,127 3/1966 Sebba ..... 209/166 X

Primary Examiner—Robert Halper

[57] ABSTRACT

A froth flotation method for the recovery of copper, nickel, cobalt, oxide, silicate, sulfide, arsenide, and antimonide minerals from their ores over iron sulfides, silica and silicates, as well as for the recovery of silicate minerals of lithium, sodium, potassium, and caesium over silica and ferromagnesian silicates, and for the recovery of potassium halides and sulfates over sodium and magnesium halides and sulfates, strontium, and barium sulfates and carbonates, which comprises; subjecting the comminuted ore of aforesaid metals and minerals to froth flotation process in the presence of nitrous acid and an effective amount of a combination of quaternary phosphonium nitrite and ternary phosphine dinitrite, and potassium, sodium, ammonium nitrite, calcium, and barium dinitrite; the indicated compounds provide selectivity and recovery of aforesaid metal and mineral values.

11 Claims, No Drawings

FROTH FLOTATION METHOD FOR THE  
RECOVERY OF MINERALS BY MEANS OF  
QUATERNARY PHOSPHONIUM NITRITES AND  
TERNARY PHOSPHINE DINITRITES

This invention relates to a new class of complexes of Werner's type in which unipositive and dipositive metals in their nitrite and dinitrite salts are replaced by their organic equivalents, the unipositive quaternary phosphonium radical, and the dipositive ternary phosphine radical. Both radicals form in combination with nitrous acid and metals at the mineral surface of hereinafter said minerals undissociable complexes of triple nitrite type with frothing properties. The triple nitrites of this invention comprise the alkylhydroxylalkyl phosphonium and alkylhydroxylalkyl phosphine radicals. The aforesaid radicals always represent two metals in the respective nitrite complexes wherein each of the two metals is a member of a different group of metals. For example one group of metals for which the aforesaid radicals would be substituted are the alkali metals, whereas another group would be the alkaline earth metals, and some weak dipositive cations such as  $\text{Ni}^{++}$ ,  $\text{Co}^{++}$ ,  $\text{Fe}^{++}$ ,  $\text{Cu}^{++}$ ,  $\text{Pb}^{++}$ . Thus the combination of aforesaid radicals and metals at the mineral surface yielding triple nitrite complexes, being so, the third metal in said triple nitrite complexes is the metal at the mineral surface.

Besides triple nitrite complexes which are the most stable and normal in such nitrites, the only stable double nitrite is formed of potassium and cobalt which is very stable. Despite of this fact the weight of the invention is put on the triple nitrite complexes. Many double nitrite salts exist but they are not stable, or not sufficient stable to serve in froth flotation practice. Thus, the stable double nitrite being feasible only with potassium and cobalt minerals, so either potassium cation which is fixed at the mineral surface combines with ternary phosphine radical representing organic equivalent of cobalt cation, or cobalt cation which is fixed at the mineral surface combines with quaternary phosphonium radical representing organic equivalent of potassium cation by means of nitrous acid radical as complexing anion.

The complexing ability of nitrite as acid radical of a very weak acid with the aforesaid metals in respective minerals depends upon the presence of coordinated alkali metals or earth alkali metals, which in the respective case of this invention the alkali metals are represented by quaternary phosphonium unipositive cations, and the earth alkali metals are represented by ternary phosphine dipositive cations. Thus, quaternary phosphonium radical with the shortest chain length of substituted hydrocarbons, which exercises a strong alkaline reaction, may unite with nitrous radical to form stable non hydrolyzable nitrites. Analogously, the ternary phosphine radical which exercises a less strong alkaline reaction, may unite with nitrous radicals to form stable non hydrolyzable dinitrites. Both, quaternary phosphonium nitrites and ternary phosphine dinitrites readily combine with aforesaid metals at the mineral surface and nitrous acid to undissociable mineral-hydrocarbon complexes of triple nitrite type.

In triple nitrite complexes of aforesaid metals, the nature of complexing cations may be such that two different quaternary phosphonium unipositive radicals yield stable undissociable complexes at the mineral surface as is the case in flotation of cobalt minerals in

a combination of diethylethanolphosphonium nitrite and dipropylpronanolphosphonium nitrite, which represent organic equivalents of potassium and sodium cations. In case of applying ternary phosphine dipositive radicals the nature of complexing cations may be such that two different ternary phosphine dipositive radicals yield stable undissociable complexes at the mineral surface as is the case in flotation of potassium silicates which is accomplished in a combination of triethylenephosphine dinitrite and dihexanolhexylphosphine dinitrite representing organic equivalents of barium and nickel cations respectively. In most cases as the experience teaches the practicing of recovering of aforesaid metals and minerals from their ores by froth flotation process and the most satisfactory in many cases and the only way to recover certain minerals is by applying a combination of quaternary phosphonium radical and ternary phosphine radical.

In accordance with the invention one unipositive cation may be potassium, sodium, or ammonium, and one dipositive cation may be calcium, barium, copper, lead, nickel, or iron, in such cases only one organic cation is sufficient, i.e., either phosphonium unipositive cation or phosphine dipositive cation. Such practicing is satisfactory and cheaper, which is an appealing advantage. Potassium, sodium, ammonium, calcium, and barium cations are added to the mineral slurry as nitrites, copper, lead, iron, and nickel cations are added to the minerals slurry as soluble salts with the addition of nitrous acid.

Because in triple nitrites three metals form the complex, which represent three groups of very alike cations, many substitutions are possible. Namely, in triple nitrite of the composition



each of the involved metal may be replaced

1. copper by metals: iron, nickel, and cobalt;
2. lead by metals: calcium, strontium, and barium;
3. potassium by metals: ammonium, rubidium, and caesium;

The organic equivalent of aforesaid complexes are as follows:

- 45 Lead-di(-trimethylethylphosphonium-dipropylpropanolphosphine)hexanitrite  
Copper-di(-trimethylethylphosphonium-dihexylhexanolphosphine)hexanitrite  
50 Nickel-di(-tetramethylphosphonium-dipropylbutanolphosphine)hexanitrite  
Cobalt-di(-trimethylethylphosphonium-tripropylpropanolphosphonium)hexanitrite  
Lithium-di(-trimethylethylphosphonium-dioctylocantanolphosphine)hexanitrite  
55 sodium-di(-tetramethylphosphonium-dioctanoloctylphosphine)hexanitrite  
Potassium-di(-tripropylphosphine-diheptylheptanolphosphine)hexanitrite  
60 Caesium-di(-triethylphosphine-dihexylhexanolphosphine)hexanitrite  
Strontium-di(-tetraethylphosphonium-dihexylhexanolphosphine)hexanitrite  
Barium-di(-tetramethylphosphonium-dihexylhexanolphosphine)hexanitrite

65 The variations of the number of hydroxyl groups in said quaternary and ternary compounds as well as in

complexes is based on the difference of alkalinity as well as because of the different lengths of alkyl chains in the same. Thus, high alkaline and short chain quaternary phosphonium or ternary phosphine radicals preferably have not any hydroxyl group, while the longer chained and less alkaline have one, two or three hydroxyls, for, minimum one hydroxyl in each complex must be present.

These replacements do not change, or change very little the stability of complexes and their insolubility.

Thus, this invention relates to a new froth flotation method for the recovery of minerals containing lithium, sodium, potassium, caesium, strontium, barium, copper, nickel, and cobalt with a combination of nitrous acid, quaternary phosphonium nitrates and ternary phosphine dinitrites, or a combination of either phosphonium nitrite and one of aforesaid metal cations, or phosphine dinitrite and one of aforesaid metal cations.

Quaternary phosphonium nitrates and ternary phosphine dinitrites are particularly adapted for the use in highly selective froth flotation processes for recovering of oxide, silicate, sulfide, arsenide, and antimonide minerals of copper, nickel, and cobalt. The method is well adapted to silicates of lithium, sodium, potassium, and caesium, such as feldspar minerals, and particularly for sodium feldspar albite, and potassium feldspar orthoclase the microcline, furthermore, potassium mica, lithium mica, as well as potassium halides and sulfates, and particularly for alunite aluminum hydrous potassium sulfate. Furthermore, for barium minerals such as barytes, and witherite, and strontium minerals such as strontianite and celestine.

Complexes of double and triple nitrates with quaternary phosphonium unipositive cations and ternary phosphine dipositive cations yield polarly oriented non-hydrolyzable and undissociable complexes capable of forming bubbles or attaching to the bubbles of the froth provided by agitation of the pulp of mineral slurry. The said quaternary phosphonium and ternary phosphine radicals of this invention possess collecting as well as some frothing properties which simplify the froth flotation process, which is obviously an advantage.

#### THE PREFERRED EMBODIMENTS

The preferred embodiments of collectors are of the following generic formulas:

for quaternary phosphonium series      for ternary phosphine series



wherein R may be of the same constitution or to be of different constitution. Thus, R may be alkyl, alkanol; or polyhydroxyalkyl such as alkyldiol or alkyltriol, said alkyl compounds have from 1 to 8 carbon atoms, and 0 to 3 hydroxyl groups. Said quaternary phosphonium radicals comprise: monoalkyltrialkanol-, dialkylalkanol-, trialkylmomoalkanol-, tetraalkyl- phosphonium nitrite, said ternary phosphine radicals comprise: trialkanol-, monoalkyldialkanol-, dialkylmonoalkanol-, trialkyl- phosphine dinitrite. The number of hydroxyl groups for the entire complex is from 1 to 3. The aforesaid radicals, i.e., phosphonium radical represents alkali metals and ammonia, whereas phosphine radical

represents earth alkali metals, and the group of weak basic dipositive cations such as  $\text{Ni}^{++}$ ,  $\text{Co}^{++}$ ,  $\text{Fe}^{++}$ ,  $\text{Cu}^{++}$ ,  $\text{Pb}^{++}$ .

The preferred embodiments of this invention representing alkali metals are:

mono-, di-, tri-, or tetra- pentanol-pentyl-phosphonium cation

mono-, di-, tri-, or tetra- butanol-butyl-phosphonium cation

mono-, di-, tri-, or tetra- propanol-propyl-phosphonium cation

mono-, di-, tri-, or tetra- ethanol-ethyl-phosphonium cation

mono-, di-, tri-, or tetra- methanol-methyl-phosphonium cation

The preferred embodiments of this invention representing earth alkali metals are:

mono-, di-, or tri- butanol-butyl-phosphine cation

mono-, di-, or tri- propanol-propyl-phosphine cation

mono-, di-, or tri- ethanol-ethyl-phosphine cation

mono-, di-, or tri- methanol-methyl-phosphine cation

The preferred embodiments of this invention representing metal dipositive cations such as  $\text{Ni}^{++}$ ,  $\text{Co}^{++}$ ,  $\text{Fe}^{++}$ ,  $\text{Cu}^{++}$ ,  $\text{Pb}^{++}$ , are:

mono-, di-, or tri- octanol-octyl-phosphine cation

mono-, di-, or tri- heptanol-heptyl-phosphine cation

mono-, di-, or tri- hexanol-hexyl-phosphine cation

mono-, di-, or tri- pentanol-pentyl-phosphine cation

In accordance with the invention one unipositive cation may be potassium, sodium, or ammonium, and one dipositive cation may be calcium, strontium, barium, copper, lead, nickel, and iron. In such cases all of possible and useful combinations yield equally satisfactory results in recovering of aforesaid minerals from their ores.

#### SUMMARY OF THE INVENTION

The principal objective of this invention is to provide a new method of froth flotation practice.

A further objective of this invention is to provide froth flotation agents with collecting and frothing properties for collecting copper, nickel, and cobalt, oxide, silicate, sulfide, arsenide, and antimonide minerals from their ores, furthermore, aluminosilicates of lithium, sodium, potassium, and caesium, potassium halides and sulfates minerals, strontium, and barium carbonates and sulfates, from their ores. In accordance with said objectives and to the best of this applicant's knowledge the said objectives have not been accomplished in the past. Furthermore, the applicant has discovered that most gangue minerals are unaffected by collectors of this invention. Hence a method for obtaining a highly selective concentration of metal or mineral values of aforesaid minerals from their ores in froth concentrates is provided.

The froth flotation of aforesaid minerals from their ores by serving with the present invention is carried out in accordance with good flotation practice and usually, though not always, involves flotation in rougher cells, followed by one or several cleanings of the rougher concentrate. The reagents are effective in small amount and the promotion is sufficiently persistent so

that it is possible to carry out rougher and cleaner flotation with a single addition of the reagents at the beginning of the operation. On the other hand, it is sometimes advantageous to use stage addition of reagents. Pulp densities are in general the same as in other applications of froth flotation practice, i.e., about 15 to 30 percent of solids by weight.

The above discussion as well as the disclosure illus-

The flotation tests were accomplished with sized sample passing 120 mesh sieve, in a 50 grams flotation cell with 10 grams of a mixture of ullmannite and chloanthite, and 40 grams of a mixture of sulfide minerals such as pyrite and gatena. The reagents were added dropwise. These flotation tests gave froth concentrates in which the recovery was estimated by microscopic count.

| Example | Collectors used                                                          | Auxiliary agents                  | Nickel Recovery percent |
|---------|--------------------------------------------------------------------------|-----------------------------------|-------------------------|
| 5       | Diethylmethanolphosphonium nitrite<br>Diethylmethanolphosphine dinitrite | Nitrous acid                      | 88                      |
| 6       | Diethylmethanolphosphonium nitrite                                       | Barium dinitrite,<br>nitrous acid | 83                      |
| 6a      | Diethylmethanolphosphine dinitrite                                       | Potassium nitrite<br>nitrous acid | 85                      |

trates my invention in a broad and general way; for a detailed illustration thereof the examples of the preferred embodiments are set forth below.

The procedure in performing laboratory examples was of the same manipulation as follows:

The flotation tests for the recovery of copper ores.

The flotation tests were accomplished with sized sample passing 120 mesh sieve, in a 50 grams flotation cell with 50 grams of a copper ore mixed of chalcopy-

The flotation tests for the recovery of cobalt minerals.

The flotation tests were accomplished with sized samples passing 120 mesh sieve in a 50 grams flotation cell with 10 grams of a mixture of cobaltite and smaltite, and 40 grams of a mixture of iron, lead, zinc, and copper sulfides. The reagents were added dropwise. These flotation tests gave concentrates in which the recovery was estimated by microscopic count.

| Example | Collectors used                                                           | Auxiliary agents                   | Cobalt Recovery percent |
|---------|---------------------------------------------------------------------------|------------------------------------|-------------------------|
| 7       | Triethylmethanolphosphonium nitrite<br>Tributylbutanolphosphonium nitrite | Nitrous acid                       | 85                      |
| 8       | Tributylbutanolphosphonium nitrite                                        | Potassium nitrite,<br>nitrous acid | 82                      |

rite and covellite and predominantly pyrite, in Examples 1 and 2, and a copper ore mixed of chrysocolla and malachite in gangue material composed of iron oxide, some pyrite, quartz, and calcium carbonate in Example 3 and 4. The reagents were added dropwise. These flotation tests gave froth concentrates in which the recovery was estimated by microscopic count.

The flotation tests for the recovery of lepidolite mineral, lithium mica.

The flotation tests were accomplished with sized samples passing 100 mesh sieve, in a 50 grams flotation cell with 5 grams of lepidolite and 45 grams of microcline. The reagents were added dropwise. These flotation tests gave froth concentrates in which the recovery

| Example | Collectors used                                                                                                    | Auxiliary agents                                                                      | Copper recovery percent |
|---------|--------------------------------------------------------------------------------------------------------------------|---------------------------------------------------------------------------------------|-------------------------|
| 1       | Trimethylmethanolphosphonium nitrite<br>Dipentylpentanolphosphine dinitrite                                        | Nitrous acid                                                                          | 93                      |
| 2       | Dipentylpentylphosphine dinitrite                                                                                  | Potassium nitrite<br>Nitrous acid                                                     | 90                      |
| 3       | Trimethylmethanolphosphonium nitrite<br>Dipentylhexanolphosphine dinitrite<br>Trimethylmethanolphosphonium nitrite | Nitrous acid<br>FeSO <sub>4</sub> , Ba(NO <sub>3</sub> ) <sub>2</sub><br>nitrous acid | 89                      |
| 4       |                                                                                                                    |                                                                                       | 87                      |

The flotation tests for the recovery of nickel ores.

was estimated by microscopic count.

| Example | Collectors used                                                     | Auxiliary agents                                      | Lepidolite recovery percent |
|---------|---------------------------------------------------------------------|-------------------------------------------------------|-----------------------------|
| 9       | Tetraethylphosphonium nitrite<br>Diocetylhexanolphosphine dinitrite | Nitrous acid                                          | 92                          |
| 10      | Diocetylhexanolphosphine dinitrite                                  | Potassium nitrite<br>nitrous acid                     | 90                          |
| 11      | Triethylmethanolphosphonium nitrite                                 | FeSO <sub>4</sub> , Ba(NO <sub>3</sub> ) <sub>2</sub> | 90                          |

7  
-continued

8

| Example | Collectors used                     | Auxiliary agents | Lepidolite recovery percent |
|---------|-------------------------------------|------------------|-----------------------------|
| 11      | Triethyllethanolphosphonium nitrite | Nitrous acid     | 95                          |

The flotation tests for the recovery of albite, sodium feldspar.

The flotation tests were accomplished with sized samples passing 100 mesh sieve, in a 50 grams flotation cell with 25 grams of albite, and 25 grams of a mixture of quartz, mica sericite, orthoclase and plagioclase. The reagents were added dropwise. These flotation tests gave concentrates in which the recovery was estimated by microscopic count.

10

The flotation tests for the recovery of sylvine, potassium chloride.

The flotation tests were accomplished with sized samples passing 48 mesh sieve, in a 50 grams flotation cell with 25 grams of sylvine and 25 grams of sodium halide in a saturated brine. The reagents were added dropwise. These froth flotation tests gave froth concentrates in which the recovery was accomplished by chemical analysis.

| Example | Collectors used                     | Auxiliary agents                                      | Albite recovery percent |
|---------|-------------------------------------|-------------------------------------------------------|-------------------------|
| 12      | Triethyllethanolphosphonium nitrite | Nitrous acid                                          | 95                      |
| 13      | Diocetylhexanolphosphine dinitrite  | FeSO <sub>4</sub> , Ba(NO <sub>3</sub> ) <sub>2</sub> | 92                      |
| 14      | Triethyllethanolphosphonium nitrite | nitrous acid                                          | 93                      |
|         | Diocetylhexanolphosphine dinitrite  | Potassium nitrite                                     |                         |
|         |                                     | nitrous acid                                          |                         |

| Example | Collectors used                      | Auxiliary agents                                      | Sylvine recovery percent |
|---------|--------------------------------------|-------------------------------------------------------|--------------------------|
| 18      | Tripropylpropanolphosphonium nitrite | Nitrous acid                                          | 92                       |
| 19      | Diocetylhexanolphosphine dinitrite   | FeSO <sub>4</sub> , Ba(NO <sub>3</sub> ) <sub>2</sub> | 85                       |
| 20      | Tripropylpropanolphosphonium nitrite | nitrous acid                                          | 88                       |
|         | Diocetylhexanolphosphine dinitrite   | Sodium nitrite                                        |                          |
|         |                                      | nitrous acid                                          |                          |

The flotation tests for the recovery of orthoclase, potassium feldspar.

The flotation tests were accomplished with sized samples passing 100 mesh sieve in a 50 grams flotation cell with 25 grams of orthoclase and 25 grams of a mixture of quartz, biotite, and plagioclase. The reagents were added dropwise. These flotation tests gave forth concentrates in which the recovery was estimated by microscopic count.

The flotation tests for the recovery of pollucite, cesium-sodium feldspar.

The flotation tests were accomplished with sized samples passing 100 mesh sieve in a 50 grams flotation cell with 5 grams of pollucite and 45 grams of orthoclase and microcline. The reagents were added dropwise. These flotation tests gave froth concentrates in which the recovery was estimated by microscopic count.

| Example | Collectors used                     | Auxiliary agent                                       | Orthoclase recovery percent |
|---------|-------------------------------------|-------------------------------------------------------|-----------------------------|
| 15      | Dipropylpropanolphosphine dinitrite | Nitrous acid                                          | 93                          |
| 16      | Dihexylhexanolphosphine dinitrite   | FeSO <sub>4</sub> , Ba(NO <sub>3</sub> ) <sub>2</sub> | 91                          |
| 17      | Triethyllethanolphosphonium nitrite | nitrous acid                                          | 93                          |
|         | Dihexylhexanolphosphine dinitrite   | Calcium dinitrite                                     |                             |
|         |                                     | nitrous acid                                          |                             |

| Example | Collectors used                     | Auxiliary agents                                      | pollucite recovery percent |
|---------|-------------------------------------|-------------------------------------------------------|----------------------------|
| 21      | Dipropylpropanolphosphine dinitrite | Nitrous acid                                          | 85                         |
| 22      | Dihexanolhexylphosphine dinitrite   | Barium dinitrite                                      | 87                         |
| 23      | Dihexanolhexylphosphine dinitrite   | nitrous acid                                          | 86                         |
|         | Dipropylpropanolphosphine dinitrite | FeSO <sub>4</sub> , Ba(NO <sub>3</sub> ) <sub>2</sub> |                            |

-continued

| Example      | Collectors used | Auxiliary agents | pollucite recovery percent |
|--------------|-----------------|------------------|----------------------------|
| nitrous acid |                 |                  |                            |

The flotation tests for the recovery of celestine, Strontium sulfate.

The flotation tests were accomplished with sized samples passing 100 mesh sieve in a 50 grams flotation cell with 50 grams of celestine ore mixed with carboniferous schist. The reagents were added dropwise. These flotation tests gave froth concentrates in which the recovery was estimated by microscopic count.

surface of said metals mineral-hydrocarbon complexes; both components of said complexes have the formula:



| Example | Collectors used                      | Auxiliary agents                                                     | Celestine recovery percent |
|---------|--------------------------------------|----------------------------------------------------------------------|----------------------------|
| 24      | Trimethylmethanolphosphonium nitrite | Nitrous acid                                                         | 92                         |
| 25      | Dihexylhexanolphosphine dinitrite    | FeSO <sub>4</sub> , Ba(NO <sub>2</sub> ) <sub>2</sub> , nitrous acid | 88                         |
| 26      | Dihexylhexanolphosphine dinitrite    | Potassium nitrite nitrous acid                                       | 88                         |

The flotation tests for the recovery of barytes, barium sulfate.

The flotation tests were accomplished with sized samples passing 120 mesh sieve, in a 50 grams flotation cell with 50 grams barytes ore mixed with pyrite and schist. The reagents were added dropwise. These flotation tests gave froth concentrates in which the recovery was estimated by microscopic count.

in which R may be of the same constitution or to be of different constitution, R is selected from the group consisting of alkyl, or alkanol, alkyldiol or alkyltriol, said R's containing from 1-8 carbon atoms, the number of hydroxyl groups furnished by the combinations of said collectors being 0 to 3, the number of said hydroxyl groups in said mineral hydrocarbon complexes

| Example | Collectors used                     | Auxiliary agents                                                     | Barytes recovery percent |
|---------|-------------------------------------|----------------------------------------------------------------------|--------------------------|
| 27      | Trimethylbutanolphosphonium nitrite | Nitrous acid                                                         | 94                       |
| 28      | Dihexylhexanolphosphine dinitrite   | FeSO <sub>4</sub> , Ba(NO <sub>2</sub> ) <sub>2</sub> , nitrous acid | 92                       |
| 29      | Dihexylhexanolphosphine dinitrite   | Potassium nitrite nitrous acid                                       | 94                       |

I claim:

1. A method of beneficiating ores selected from the group consisting of oxide, silicate, sulfide, arsenide, and antimonide of copper, nickel and cobalt, and minerals selected from the group consisting of lithium, sodium, potassium and caesium silicates, halides and sulfates, barium and strontium sulfates and carbonates by froth flotation process to produce a froth concentrate of desired metal or mineral value which comprises; effecting froth flotation of said ores and minerals in the presence of nitrous acid and collectors consisting of a combination of quaternary phosphonium nitrite and ternary phosphine dinitrite, or a combination of two different quaternary phosphonium nitrates, or a combination of two different phosphine dinitrites, or a combination of quaternary phosphonium nitrite and either sodium, potassium, and ammonium nitrates, or calcium, strontium, barium, and iron dinitrites, or a combination of ternary phosphine dinitrites and either sodium, potassium, and ammonium nitrates, or calcium, strontium, barium, and iron dinitrites, said compounds in conjunction with nitrous acid forming at the mineral

being 1 to 3, the shorter chain R's of said phosphonium nitrates and phosphine dinitrites having zero hydroxyl groups, the longer R's of said phosphonium nitrates and phosphine dinitrites having 1-3 hydroxyl groups, said complexes attaching to bubbles provided by agitating the pulp of mineral slurry; and recovering a froth concentrate relatively rich in the desired metal or mineral value, leaving tailings relatively poor in the desired metal or mineral value.

2. A method according to claim 1, of beneficiating ores selected from the group consisting of oxide, silicate, sulfide, arsenide, and antimonide of copper by froth flotation process to produce a copper concentrate which comprises; effecting froth flotation of aforesaid ores in the presence of nitrous acid and collectors comprising a combination of quaternary phosphonium nitrite and ternary phosphine dinitrite, or a combination of ternary phosphine dinitrite and potassium nitrite, or a combination of quaternary phosphonium nitrite and iron dinitrite, R in said phosphonium nitrite contains 1 to 3 carbon atoms, and R in said phosphine dinitrite contains 5 to 7 carbon atoms, said collectors in con-

junction with nitrous acid and copper at the mineral surface forming mineral-hydrocarbon undissociable complexes attaching to bubbles provided by agitating the pulp of mineral slurry; and recovering a froth concentrate relatively rich in copper metal value.

3. A method according to claim 1 of beneficiating ores selected from the group consisting of oxide, silicate, sulfide, arsenide, and antimonide of nickel by froth flotation process to produce a nickel froth concentrate which comprises; effecting froth flotation of aforesaid ores in the presence of nitrous acid and collectors comprising a combination of quaternary phosphonium nitrite and ternary phosphine dinitrite, or a combination of quaternary phosphonium nitrite and barium dinitrite, or a combination of ternary phosphine dinitrite and potassium nitrite, R in said phosphonium nitrite contains 2 to 3 carbon atoms, and R in said phosphine dinitrite contains 2 to 4 carbon atoms, collectors in conjunction with nitrous acid and cobalt at the mineral surface forming mineral-hydrocarbon undissociable complexes attaching to bubbles provided by agitating the pulp of mineral slurry; and recovering a froth concentrate relatively rich in nickel metal value, leaving tailings relatively poor in nickel metal value.

4. A method according to claim 1 of beneficiating ores selected from the group consisting of oxide, sulfide, arsenide, and antimonide of cobalt by froth flotation process to produce a cobalt froth concentrate which comprises; effecting froth flotation of aforesaid ores in the presence of nitrous acid and collectors comprising a combination of two different quaternary phosphonium nitrates, or a combination of quaternary phosphonium nitrite and potassium or sodium nitrite, of which R in one phosphonium nitrite contains from 1 to 2 carbon atoms, and in the other phosphonium nitrite the number of carbon atoms in R is from 2 to 4, said collectors in conjunction with nitrous acid and cobalt at the mineral surface forming mineral-hydrocarbon undissociable complexes attaching to bubbles provided by agitating the pulp of mineral slurry; and recovering a froth concentrate relatively rich in cobalt metal value, leaving tailings relatively poor in cobalt metal value.

5. A method according to claim 1 of beneficiating ores selected from the group of lithium silicates by froth flotation process to produce a lithium froth concentrate which comprises; effecting froth flotation of the ore in the presence of nitrous acid and collectors comprising a combination of quaternary phosphonium nitrite and either ternary phosphine dinitrite or iron dinitrite, or a combination of ternary phosphine dinitrite and potassium nitrite, R in said phosphonium nitrite contains 1 to 2 carbon atoms, and R in said phosphine dinitrite contains 6 to 8 carbon atoms, said collectors in conjunction with nitrous acid and lithium at the mineral surface forming mineral-hydrocarbon undissociable complexes attaching to bubbles provided by agitating the pulp of mineral slurry; and recovering a froth concentrate relatively rich in lithium silicate value, leaving tailings relatively poor in lithium silicate value.

6. A method according to claim 1 of beneficiating ores selected from the group of sodium silicates by froth flotation process to produce a sodium silicate concentrate which comprises; effecting froth flotation of the ore in the presence of nitrous acid and collectors comprising a combination of quaternary phosphonium nitrite and either ternary phosphine dinitrite or iron

dinitrite, or a combination of ternary phosphine dinitrite and potassium nitrite, R in said phosphonium nitrite contains 1 to 3 carbon atoms, and R in said phosphine dinitrite contains 6 to 8 carbon atoms, said collectors in conjunction with nitrous acid and sodium at the mineral surface forming mineral-hydrocarbon undissociable complexes attaching to bubbles provided by agitating the pulp of mineral slurry; and recovering a froth concentrate relatively rich in sodium silicate value, leaving tailings relatively poor in sodium silicate value.

7. A method according to claim 1 of beneficiating ores selected from the group of potassium silicates by froth flotation process to produce a potassium silicate froth concentrate which comprises; effecting froth flotation of the ore in the presence of nitrous acid and collectors comprising a combination of two different ternary phosphine dinitrites, combination of one ternary phosphine dinitrite and either calcium or iron dinitrite R in one phosphine dinitrite contains 2 to 4 carbon atoms, and R in the other phosphine dinitrite contains 6 to 7 carbon atoms, said collectors in conjunction with nitrous acid and potassium at the mineral surface, forming mineral-hydrocarbon undissociable complexes attaching to bubbles provided by agitating the pulp of mineral slurry; and recovering a froth concentrate relatively rich in potassium silicate value, leaving tailings relatively poor in potassium silicate value.

8. A method according to claim 1 of beneficiating ores selected from the group of potassium halides and sulfates by froth flotation process to produce a potassium halide or sulfate froth concentrate which comprises; effecting froth flotation of the ore in the presence of nitrous acid and collectors comprising a combination of quaternary phosphonium nitrite and either ternary phosphine dinitrite or iron dinitrite, or a combination of ternary phosphine dinitrite and sodium nitrite, R in said phosphonium nitrite contains 2 to 4 carbon atoms, and R in said phosphine dinitrite contains 6 to 8 carbon atoms, said collectors in conjunction with nitrous acid and potassium at the mineral surface forming mineral-hydrocarbon undissociable complexes attaching to bubbles provided by agitating the pulp of mineral slurry; and recovering a froth concentrate relatively rich in potassium halide or sulfate value, leaving tailings relatively poor in potassium halide or sulfate value.

9. A method according to claim 1 of beneficiating ores selected from the group of caesium silicates by froth flotation process to produce a caesium silicate froth concentrate which comprises; effecting froth flotation of the ore in the presence of nitrous acid and collectors comprising a combination of two different ternary phosphine dinitrite, or a combination of ternary phosphine dinitrite and either barium or iron dinitrite, R in one of said phosphine dinitrite contains from 2 to 4, and in the other phosphine dinitrite 5 to 7 carbon atoms, said collectors in conjunction with nitrous acid and caesium at the mineral surface forming mineral-hydrocarbon undissociable complexes attaching to bubbles provided by agitating the pulp of mineral slurry; and recovering a froth concentrate relatively rich in caesium silicate value, leaving tailings relatively poor in caesium silicate value.

10. A method according to claim 1 of beneficiating ores selected from the group of strontium sulfate and carbonate by froth flotation process to produce a strontium sulfate or carbonate froth concentrate which com-

13

prises; effecting froth flotation of the ore in the presence of nitrous acid and collectors comprising a combination of quaternary phosphonium nitrite and either ternary phosphine dinitrite or iron dinitrite, or a combination of ternary phosphine dinitrite and potassium nitrite, R in said phosphonium nitrite contains 2 to 3 carbon atoms, and R in said ternary phosphine dinitrite contains 5 to 7 carbon atoms, said collectors in conjunction with nitrous acid and strontium at the mineral surface forming mineral-hydrocarbon undissociable complexes attaching to bubbles provided by agitating the pulp of mineral slurry; and recovering a froth concentrate relatively rich in strontium sulfate or carbonate value leaving tailings relatively poor in strontium sulfate or carbonate value.

11. A method according to claim 1 of beneficiating ores selected from the group of barium sulfate or carbonate by froth flotation process to produce a barium

14

sulfate or carbonate froth concentrate which comprises; effecting froth flotation of the ore in the presence of nitrous acid and collectors comprising a combination of quaternary phosphonium nitrite and either ternary phosphine dinitrite or iron dinitrite, or a combination of ternary phosphine dinitrite and potassium nitrite, R in said phosphonium nitrite contains 1 to 2 carbon atoms, and R in said ternary phosphine dinitrite contains 6 to 8 carbon atoms, said collectors in conjunction with nitrous acid and barium at the mineral surface forming mineral-hydrocarbon undissociable complexes attaching to bubbles provided by agitating the pulp of mineral slurry; and recovering a froth concentrate relatively rich in barium sulfate or carbonate value leaving tailings relatively poor in barium sulfate or carbonate value.

\* \* \* \*

20

25

30

35

40

45

50

55

60

65